

March 26, 1968

F. E. BATTON

3,375,159

PARADICHLOROBENZENE BLOCK

Filed Sept. 17, 1964



INVENTOR

FRANCIS E. BATTON

BY

*Christopher A. Spencer*  
ATTORNEYS

1

3,375,159

**PARADICHLOROBENZENE BLOCK**

Francis E. Batton, New Martinsville, W. Va., assignor to Pittsburgh Plate Glass Company, Pittsburgh, Pa., a corporation of Pennsylvania

Filed Sept. 17, 1964, Ser. No. 397,296

5 Claims. (Cl. 167—30)

**ABSTRACT OF THE DISCLOSURE**

A method of improving the strength of scented paradichlorobenzene blocks or cakes is described in which the paradichlorobenzene block or cake containing the scenting agent is passed through a heat source and heated to a temperature and for a period of time sufficient to coalesce the particles on the surface of the block or cake without deforming it. Specifically the heat treatment is conducted at such temperatures and for periods of time sufficient to prevent the block from achieving a temperature of 127° F. in the center thereof. Various methods of heating the block are described. A specific example on electrical heating is shown.

The present invention relates to a method of improving the strength of scented, compacted crystals of paradichlorobenzene. More particularly, the present invention relates to a method of improving the strength of scented paradichlorobenzene blocks, and to a new article of manufacture.

In the manufacture of paradichlorobenzene cakes, bars, and other physical configurations of paradichlorobenzene crystals, it is customary to place in the cake a scenting agent or perfume to provide in the finished product a paradichlorobenzene packet of compressed crystals having a pleasant odor. In conducting this scenting process the liquid perfume or scenting material is mixed with the paradichlorobenzene crystals prior to compressing them into the desired physical form. After thorough mixing of the crystals with the scenting agent, the crystals are then compacted or compressed to the desired shape in a pressing machine by applying suitable pressure to the scented crystals in a die. Typical pressures are from 300 to 2,000 p.s.i.

One disadvantage encountered in scenting or perfuming paradichlorobenzene crystals which are made into cakes or blocks has been that the finished product loses a considerable amount of its normal strength due to the presence of the perfume or scenting materials. All perfumes employed for this purpose have this effect on the finished product to a greater or lesser degree. The net result of the employment of these materials in paradichlorobenzene compressed crystal bodies is the same however, their normal strength, that is, the strength of the compressed crystal bodies without such perfumes, is markedly reduced. Thus, it is quite common for a finished paradichlorobenzene block not containing any scented material to have a breaking pressure on the order of 700 to 800 p.s.i. the first day after manufacture. A similar block containing a scenting material will have a breaking pressure of something on the order of 200 to 300 p.s.i. In the shipping and handling of the finished blocks or cakes of scented paradichlorobenzene, considerable breakage is thus encountered. While the presence of scenting materials in paradichlorobenzene blocks is a desirable feature in reducing the unpleasant odor of unscented crystals of paradichlorobenzene and imparts a pleasant odor for certain applications, for example, as sanitary cakes for toilet bowls, for deodorizing closets, etc. the decreased strength of such scented materials and the subsequent breakage detracts from their desirability.

2

In accordance with the instant invention a method has been devised whereby paradichlorobenzene cakes may be formed with the scenting material and a considerable reduction in the loss of strength normally encountered readily achieved. In accordance with the present invention paradichlorobenzene crystals are admixed with the scenting materials to be employed. After the scenting material has been thoroughly mixed with the paradichlorobenzene crystals, the crystals are compacted in a conventional manner and then contacted with a heat source at a high enough temperature and for a sufficient period of time to cause the paradichlorobenzene crystals to coalesce or fuse at least on the surface of the block. In this manner a compacted mass of paradichlorobenzene is provided which maintains a high breaking strength for a considerable period of time, while surprisingly during the heating operation little or no weight loss of the paradichlorobenzene compacted crystals occurs.

When conducting the heat treating step of the instant invention recourse of various types of heat may be had. It is preferred that the heat be applied by an electrical source, preferably through the utilization of heat lamps or heating panels or other similar electrical devices. While this mode of heat application is preferred, other sources of heat may be employed. Thus, heat supplied indirectly from gas fired furnaces, light sources, resistance wires, and other similar heating mechanisms may be readily employed. It would be undesirable of course to utilize a heat source which directly impinged a flame on the paradichlorobenzene crystals and thus direct firing of the cakes with a flame is to be avoided.

The temperatures to which the paradichlorobenzene compacted crystals are subjected will vary considerably depending upon the length of time that it is desired to expose the cake or block to the heat source. Generally, temperatures may range between 120° F. up to about 200° F. It is preferable in applying heat to the compacted crystals of scented paradichlorobenzene that the heat be applied in the range of between about 150° F. and about 175° F. The total quantity of heat applied to the block during treatment should be of course below that which would cause deformation of the block by melting of the paradichlorobenzene crystals. A temperature of over 127° F. in the center of the paradichlorobenzene block being treated is to be avoided.

The length of time to which the scented, compacted paradichlorobenzene crystals are exposed to the heat source will vary considerably depending upon the size of the block or cakes employed, the temperature used and other similar considerations. Generally, the time of treatment may range from between 30 seconds up to about 15 minutes or more. Preferably, heat treatments in the range of 150° F. to 175° F. will be conducted at a period of time ranging between 60 seconds to about 10 minutes.

It is found in operating in accordance with the above parameters that paradichlorobenzene cakes which have been scented with perfumes will form a hard cake having considerably more strength than a paradichlorobenzene scented cake which has not been heat treated. Surprisingly the weight loss occurring during the heat treatment will normally be about one half of 1 percent of the total weight of the block subjected to the heat treatment. Thus, the advantages gained by increased strength greatly outweigh any weight loss as minute as those encountered during the heat treating steps herein set forth.

For a more complete understanding of the present invention, reference is made to the following example, which is illustrative with one mode of practicing the present invention.

**3**  
*Example*

The equipment used for the heat treatment was a 24 inch wide belt conveyor 14 foot in length. This conveyor was surrounded by an oven 24 inches wide and 12 foot in length. The oven was equipped with six, 16 by 24 inch Corning glass heating panels rated at 2500 watts and 230 volts. The panels were evenly spaced over the 12 foot length of oven and were mounted 2½ inches above the canvas conveying belt. For the heat treating test, the temperature in the oven was controlled at 165° F. by a rheostat on the power supply to the panels. The scented blocks of paradichlorobenzene 2.25 inches in diameter and 0.75 inch thick were placed flat on the conveyor and carried through the oven at a feed rate of 8 feet per minute. Since only one side of the block was treated this way, the blocks were then passed through the oven a second time and the unexposed side of the block was treated. The total exposure time was 3 minutes and the oven temperature was 165° F. None of the blocks treated in this manner were deformed in shape after treatment. Utilizing these procedures, a series of four runs were made on paradichlorobenzene blocks prepared by mixing 6 ounces of various commercial perfumes with paradichlorobenzene crystals and subsequently blocking these scented crystals in a blocking machine by compression. The blocks were sent through the furnace on the conveyor belt in the manner indicated above and upon completion of the exposure were tested for their breaking strength. The results of these tests are set forth in the table below. As a control to determine the effectiveness of the heat treatment, paradichlorobenzene blocks manufactured from the same perfumes and in the same manner as those treated above but not subjected to the heat treating step were compared for their breaking strength at intervals from 1 to 20 days. The results of these tests are shown below in Table II.

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

490

500

510

520

530

540

550

560

570

580

590

600

610

620

630

640

650

660

670

680

690

700

710

720

730

740

750

760

770

780

790

800

810

820

830

840

850

860

870

880

890

900

910

920

930

940

950

960

970

980

990

1000

4

While the invention has been described with reference to certain specific examples, it is to be understood that it is not to be so limited except insofar as appears in the accompanying claims.

5

I claim:

1. A method of improving the strength of scented, compacted crystalline paradichlorobenzene comprising contacting said scented, compacted crystalline paradichlorobenzene with a source of heat at a temperature sufficiently high and for a period of time sufficient to cause the paradichlorobenzene crystals to coalesce at least on the surface but insufficient to cause the temperature in the center of the block to exceed 127° F.

2. A method of improving the strength of scented, compacted paradichlorobenzene cake comprising contacting said cake with a source of heat at a temperature of between 120° F. to 200° F. for a period of time ranging from 30 seconds to 15 minutes but insufficient to cause the temperature in the center of the block to exceed 127° F.

3. The method of claim 2 wherein the temperature ranges between 150° F. and 175° F. in a period of time ranging between 60 seconds to 10 minutes.

4. A method of improving the strength of scented paradichlorobenzene blocks comprising contacting said blocks of paradichlorobenzene with a source of heat at a temperature of at least 165° F. for a period of at least 3 minutes but insufficient to cause the temperature in the center of the block to exceed 127° F.

5. A scented paradichlorobenzene block prepared in the manner set forth in claim 4.

TABLE I

| Compound                                      | Oz. Perfume/<br>100# Paradichlorobenzene<br>Added | Age of Block (days) |     |     |     |     |     |     |    |    |  |
|-----------------------------------------------|---------------------------------------------------|---------------------|-----|-----|-----|-----|-----|-----|----|----|--|
|                                               |                                                   | 0                   | 1   | 2   | 3   | 4   | 5   | 10  | 15 | 20 |  |
| Breaking Pressure (p.s.i.)                    |                                                   |                     |     |     |     |     |     |     |    |    |  |
| Felton Rose <sup>1</sup>                      | 6                                                 | 350                 | 400 | 420 | 475 | 450 |     |     |    |    |  |
| M, M&R Spice <sup>1</sup>                     | 6                                                 | 300                 | 325 | 400 | 400 | 340 |     |     |    |    |  |
| Narve, Pine <sup>1</sup>                      | 6                                                 | 340                 | 400 |     | 350 | 300 |     |     |    |    |  |
| G&D, <sup>1</sup> Nectar Bouquet <sup>2</sup> | 6                                                 | 330                 | 300 |     |     | 580 | 560 | 450 |    |    |  |

<sup>1</sup> Blocks annealed at 165° F. for 180 seconds.

TABLE II

| Compound                         | Oz. Perfume/<br>100# Paradichlorobenzene<br>Added | Age of Block (days) |     |     |     |     |     |     |     |     |  |
|----------------------------------|---------------------------------------------------|---------------------|-----|-----|-----|-----|-----|-----|-----|-----|--|
|                                  |                                                   | 0                   | 1   | 2   | 3   | 4   | 5   | 10  | 15  | 20  |  |
| Breaking Pressure (p.s.i.)       |                                                   |                     |     |     |     |     |     |     |     |     |  |
| Felton Rose                      | 6                                                 | 275                 | 120 | 90  | 90  | 100 |     |     |     |     |  |
| M, M&R Spice                     | 6                                                 | 200                 | 120 | 140 | 120 | 100 | 90  |     |     |     |  |
| Narve, Pine                      | 6                                                 | 310                 | 260 | 190 | 130 | 110 | 110 | 110 | 110 | 110 |  |
| G&D, Nectar Bouquet <sup>2</sup> | 6                                                 | 240                 | 120 |     |     | 100 | 90  | 90  | 90  | 90  |  |

As can be readily seen from the examination of the two tables, the paradichlorobenzene blocks which had been heat treated exhibited, immediately after treatment, significant increases in strength over those which did not receive any heat treatment. After a period of one day the comparison shows an even greater difference between the two sets of scented blocks.

As can be readily seen from the above results, by exposing scented paradichlorobenzene blocks to the heat treatment hereinabove described, superior scented paradichlorobenzene blocks are prepared which possess strength qualities in this product heretofore not attainable.

## References Cited

## UNITED STATES PATENTS

|           |         |             |           |
|-----------|---------|-------------|-----------|
| 1,346,337 | 7/1920  | Roark       | 167—30    |
| 1,515,364 | 11/1924 | Roark       | 167—30    |
| 2,328,690 | 9/1943  | Steele      | 167—30    |
| 2,789,078 | 4/1957  | Trusler     | 167—33    |
| 2,081,236 | 5/1937  | Hinegardner | 260—650   |
| 2,527,606 | 10/1950 | Webb        | 260—650   |
| 2,843,914 | 7/1958  | Koury       | 264—125 X |

70 ALEXANDER H. BRODMERKEL, Primary Examiner.

P. E. ANDERSON, Assistant Examiner.